

# UNITED STATES PATENT OFFICE.

CHARLES VICKERS, OF NIAGARA FALLS, NEW YORK, ASSIGNOR TO THE TITANIUM ALLOY MANUFACTURING COMPANY, OF NEW YORK, N. Y., A CORPORATION OF MAINE.

## ALLOY.

1,264,459.

Specification of Letters Patent. Patented Apr. 30, 1918.

No Drawing.

Application filed September 27, 1916. Serial No. 122,344.

To all whom it may concern:

Be it known that I, CHARLES VICKERS, a subject of the King of Great Britain, and a resident of Niagara Falls, in the county of 5 Niagara and State of New York, have invented certain new and useful Improvements in Alloys, of which the following is a specification.

My present invention relates to alloys of 10 copper with aluminium, commonly known as "aluminium-bronzes," and its objects comprise the production, by aid of my herein-after described, novel procedures and additions, of novel alloys of essentially the type 15 referred to, but distinguishable from the latter in that the ratio of hardness and rigidity on the one hand to ductility, elongation and yield on the other is, in my said. alloys, novelly and importantly smaller than, 20 I believe, heretofore attained or attainable.

Aluminium bronzes have proved disappointing, in many instances, because of the hitherto impossibility of combinedly imparting thereto not only the ductility to be expected, but also the hardness and rigidity indispensable for certain uses. They have hitherto usually proved either so highly ductile and soft as to be too easily deformable 25 30 to be sufficiently hardened for such purposes, as by, as heretofore, increasing their content of aluminium, have proved equally unavailable because thereby rendered insufficiently soft and ductile. This I have found is due 35 to the sudden stiffening of the alloy which takes place during its formation whenever the aluminium content is raised above a certain limit, which I have discovered to be say about 8 per cent.

40 I have also discovered that by suitably adding iron to the said alloys, their aforesaid, and other, objectionable features, can be practically remedied, or entirely overcome, and that by proper, properly made, 45 additions of that metal the ratio of hardness, and rigidity, to ductility, elongation and yield can, within limits, be varied at will, and without impairment of the other characteristic and desired properties of the final 50 products regarded as aluminium bronzes.

I have further discovered that, while the respective percentages of the copper, aluminium, and iron, can be very considerably

varied to serve the special requirements of various special uses, the satisfactory and useful range of the iron is practically limited to from one to five per cent. of the final product or alloy, and of the aluminium from five to twelve per cent., the remainder of my aluminium bronze alloys being composed 60 essentially of copper, or its equivalent, and the results of a long series of experiments with different charges, and tests of their resulting products, indicate that aluminium bronzes containing from 7 to 8 per cent. of 65 aluminium are very greatly improved in all physical properties by my said additions thereto of from 3 to 4 per cent. of iron, so much so in fact that they can be, and have been, with entire satisfaction applied to uses 70 for which aluminium bronzes have hitherto proved unavailable.

The method resorted to for production of my novel copper-aluminium-iron alloys is, I find, of great importance as bearing upon 75 the aforesaid and other required characteristics and properties thereof. I have discovered that, thus far, my said alloys are best producible, and with the most satisfactory properties, only by the following procedure, 80 viz: I charge into the bottom of the crucible, or other container, to be employed in the melting, the iron in thin sheet form, such as tin plate, or planished sheet iron, and, of course, in the proportion required to insure 85 its percentage determined upon for the final product. Upon the iron thus charged, I further charge the required proportion of copper, and then melt these two metals, so charged, together. To this molten charge I 90 then add the required proportion of aluminium, thereby insuring that any theretofore undissolved iron shall go into the solution, and thus insure homogeneity, and other desirable properties, in the final alloy 95 product, the which, after its complete formation, I run into molds, cool, etc., as usual. One advantage of this procedure, by reason, as I believe, of the action of the aluminium upon the iron under the conditions specified, 100 is that it operates to overcome the hitherto experienced difficulties due to the reluctance of the iron to completely alloy with the copper, and from which, in alloys of copper and iron, has undesirably resulted those iron segregations in the form of nodules and of such 105

extreme hardness as to injure prohibitively the instrumentalities employed in tooling such alloys.

I am aware that prior to my invention an alloy has been described as containing .9203 copper, .0267 aluminium and .0530 iron; also an alloy containing .9399 copper, .0446 aluminium and .0149 iron neither of which alloys do I claim as constituting any part of my invention which proceeds upon my discovery that as aforesaid not less than five nor more than twelve per cent. of aluminium and not more than from three to four per cent. of iron in such alloys, the ratio of aluminium to iron being not more than two and a half to one, coöperate to not only very greatly increase ductility, elongation and yield but also and simultaneously hardness and rigidity; and that outside of these particular proportions the result is unattainable and the alloys correspondingly inferior or useless for certain purposes which my said alloys satisfactorily subserve.

Having now described my invention, what I claim as new and desire to secure by Letters Patent is the following, viz:

1. The herein described composition, or alloy, of copper, aluminium, and iron, the

aluminium constituting from seven to twelve per cent. and the iron from three to four 30 per cent. of the whole.

2. The herein described composition, or alloy, of copper, aluminium, and iron, the aluminium constituting not less than seven per cent. nor more than twelve per cent. and 35 the iron not less than three per cent. nor more than five per cent. of the whole, the proportion of the aluminium to the iron in each case being not more than two and one half to one.

3. The herein described composition, or alloy, of copper, aluminium, and iron the aluminium constituting ten per cent. and the iron four per cent. of the whole.

4. The herein described composition, or alloy, of copper, aluminium, and iron the aluminium constituting not less than seven per cent. of the whole, the iron being in each case less than the aluminium, and the proportion of aluminium to iron being not more 50 than two and one half to one.

CHARLES VICKERS.

Witnesses:

W. H. ARGUE, Jr.,  
FRANK C. KING.